

## UNITED STATES PATENT OFFICE.

SVEN JOHAN NORDSTROM, OF SAN FRANCISCO, CALIFORNIA, ASSIGNEE, BY DIRECT AND MESNE ASSIGNMENTS, TO MERCO NORDSTROM VALVE COMPANY, OF SAN FRANCISCO, CALIFORNIA, A CORPORATION OF DELAWARE.

## LUBRICANT.

No Drawing.

Application filed August 28, 1922. Serial No. 584,864.

*To all whom it may concern:*

Be it known that I, SVEN JOHAN NORDSTROM, a subject of the King of Sweden, and a resident of San Francisco, in the 5 county of San Francisco and State of California, have invented certain new and useful Improvements in Lubricants, of which the following is a specification.

The invention relates to an improvement 10 in lubricants, and more particularly to an improvement in compounds for lubricating relatively movable parts such as valves and the like which are subject to the effects of steam or high temperatures.

15 The object of the invention is to produce a lubricating compound which will preserve its body or lubricating qualities for a reasonable length of time when subjected to high temperatures and high pressure. To 20 this end, the invention consists in the improved lubricant hereinafter described and particularly pointed out in the appended claims.

In preparing my improved lubricant I 25 use a mixture of a water-insoluble calcium soap and a high flash mineral oil. Calcium soaps as heretofore prepared I found to be unsuitable for the purpose, and accordingly I have prepared a new calcium soap for use 30 in making the improved lubricant. The new calcium soap imparts to the lubricating compound the property of keeping its body or lubricating qualities while in the presence of high temperatures.

35 The calcium soap is prepared by taking substantially 780 grams of vegetable oil, preferably castor oil, and 220 grams of vegetable wax, preferably carnauba wax, and melting them together. In a separate vessel 40 500 grams of quicklime is stirred into seven liters of water and brought to a boil. The melted castor oil and carnauba wax are poured carefully into the boiling lime water so as to prevent the mixture from boiling

over. The mass is then boiled for thirty 45 minutes and is thoroughly stirred from time to time. After the mixture has settled, the water is poured off, and the residue is brought to its melting point. The mass is afterward allowed to cool and is then 50 broken into small pieces of about one-quarter inch mesh. The calcium soap as thus formed is then ground into small particles. To facilitate the grinding of the soap it is mixed with one-sixth of its weight of flake 55 graphite. The calcium soap composed as described above is insoluble in water, and therefore is particularly adapted for use as an ingredient in lubricants subjected to steam and hot water.

60 The powdered calcium soap and graphite is mixed with substantially twice its weight of railroad valve oil or some other mineral oil having a high flash point. The powder and oil are stirred cold until thoroughly 65 mixed. The mixture is then placed on a hot plate and stirred constantly until it is completely melted.

The lubricating compound, as thus prepared, is then cooled and formed into 70 sticks, as with a grease gun, and the sticks rolled in graphite. The improved lubricating compound is a stiff paste at 400° F. At 500° F. it begins to flow, and at 600° F. it has the consistency of thick molasses. It 75 will thus be recognized that the lubricant is adapted for use in the presence of steam and high temperatures generally.

Having thus described the invention 80 what I claim as new is: —

1. A lubricating compound comprising a mineral oil and a calcium soap made from castor oil, carnauba wax and quicklime.
2. A lubricating compound comprising a mixture of mineral oil and a calcium soap made from vegetable oil, vegetable wax and quicklime.

SVEN JOHAN NORDSTROM.